

# UNITED STATES PATENT OFFICE.

WILLIAM JOHN WILLIAMS, OF CAMDEN, NEW JERSEY.

## MORDANT.

SPECIFICATION forming part of Letters Patent No. 398,564, dated February 26, 1889.

Application filed August 13, 1888. Serial No. 282,612. (No specimens.)

*To all whom it may concern:*

Be it known that I, WILLIAM JOHN WILLIAMS, a subject of the Queen of Great Britain and Ireland, and a resident of Camden, 5 Camden county, New Jersey, have invented a Mode of Fixing Dye-Colors, of which the following is a specification.

My invention relates to the fixing of dye-colors upon fibers or fabrics, whether of cotton, silk, wool, jute, flax, or other material; and the object of my invention is to so treat the fibers or fabrics that the colors will be fixed thereon and that no superfluous coloring-matter will be absorbed by the fibers or fabrics, and in consequence the latter will be free 15 from "rust" or oxidation of the colors, and the colors will not come off or "crock."

I have discovered that dye-colors may be fixed on fibers or fabrics by subjecting them 20 to the action of trisodium phosphate.

In carrying out my invention the trisodium phosphate may be added directly to the dye-bath, or it may be employed in the finishing-bath, or it may be added to the water or other 25 liquid which is to be used in either of those baths, or the fabrics or fibers may be treated to the action of a solution of the trisodium phosphate before being put in the dye-bath or after they have been dyed and finished.

30 The quantity of trisodium phosphate to be used will vary with the character of the material to be dyed and with the nature of the dye used, and to some extent with other attendant conditions. A one-per-cent. solution gives 35 the desired effect—that is, it has the property of fixing the colors on the textile fabrics or fibers so as to give a dense and lasting color—and if the phosphate be used in the dye-bath it will prevent the absorption of any

40 superfluous coloring-matter in the stock, so that the fibers or fabrics will be free from rust and the colors be prevented from "crocking." Moreover, by the employment of trisodium phosphate the use of sodium sulphate (Glauber's salts) or potassium bitartrate (tartar or argol) both in the dyeing and mordanting operations may be entirely dispensed with. Owing to the strong affinity of the trisodium phosphate for the coloring-matter of 45 50 the dye-stuffs, the color is more fully precipitated and a brighter and a fuller color is ob-

tained from a smaller quantity of dye and the color is made more fast. The use of this trisodium phosphate results in great economy, for where twenty to twenty-five pounds of 55 Glauber's salts have been heretofore used eight ounces of trisodium phosphate will accomplish the purpose. So, again, the same amount of trisodium phosphate will replace two to three pounds of half-refined potassium 60 bitartrate.

I employ trisodium phosphate in place of all other phosphates because in it the phosphoric acid is fully neutralized, so that there is no free acid in the compound, nor is any produced 65 in any of the baths in which it may be used.

I am aware that many years ago the suggestion was made that alkaline phosphates should be used in dyeing operations—as, for instance, in Bowden's British Patent No. 2,764 of 1861—70 in which it was proposed to use phosphate of soda for fixing colors on cotton goods or fabrics; but the commercial phosphate of soda previous to this time has been disodium phosphate, which has been but rarely used, practically on account of drawbacks to its use hereinafter mentioned. On the other hand I have obtained highly-successful results with trisodium phosphate, effecting a saving of fifty 75 per cent. and over in the use of dye-stuff and 80 producing a better and more durable and faster color.

Trisodium phosphate has materially different and distinctive properties from disodium or other sodium phosphates. Thus compare 85 the analyses:

|                  | Disodium phosphate. | Trisodium phosphate. |
|------------------|---------------------|----------------------|
| Phosphoric acid, | 19.84               | 18.68                |
| Soda,            | 17.32               | 24.48                |
| Water,           | 62.84               | 56.84                |

90 In the dye-bath the presence of mineral salts exerts a very powerful action on the dye-stuff and frequently prevents the fabric from "taking" or absorbing the dye, and this more especially if the action of the dye-stuff, mordant, 95 or chemical reagents used as "fixers" on these mineral substances set free acid or acid salts. Most (nearly all) waters contain lime sulphate, magnesia sulphate, lime carbonate, &c. Now, disodium phosphate, reacting on these mineral 100 salts in the water, sets free sulphuric or carbonic acid, or both, (or forms acid bisulphate

and bicarbonate,) which prevent the fabric from taking up its due amount of dye and render the colors dull and poor, and at the same time waste the dye-stuff. Trisodium phosphate, on the other hand, contains nearly fifty per cent. more soda than disodium phosphate, and in reacting on these mineral salts in the water produces neutral salts, (and no free acid,) and thus enables the fabric to "take" or absorb the dye-stuff freely, producing brighter and clearer colors with a much smaller quantity of dye.

I claim as my invention—

The mode herein described of fixing colors and preventing rust and crocking in textile fibers or fabrics, said mode consisting in subjecting the fabrics or fibers to the action of trisodium phosphate.

In testimony whereof I have signed my name to this specification in the presence of two subscribing witnesses.

WM. JOHN WILLIAMS.

Witnesses:

JOHN W. PRESTWICH,  
LOUIS B. HUMPHREYS.